

## UNITED STATES PATENT OFFICE

2,128,677

## DRAWING OF GALVANIZED WIRE

Frank Jenks, Port Waratah, Newcastle, New South Wales, Australia, assignor to Rylands Brothers (Australia) Limited, Port Waratah, Newcastle, New South Wales, Australia, a corporation of New South Wales

No Drawing. Application May 22, 1937, Serial No. 144,303. In Australia July 14, 1936

3 Claims. (Cl. 205—21)

This invention consists in improvements in the process of "dry" drawing steel wire, which is "galvanized" or otherwise coated with zinc or zinc alloys either before or at an intermediate stage in the drawing passes and it has for its object the production of zinc or zinc-alloy covered steel wire by means whereby it will be caused to come from the final pass well finished with its surface clear and bright.

10 In usual practice steel wire rod is drawn in an appropriate number of passes to reduce its section to its ultimate required size and is then coated with zinc or zinc alloy. In some cases the zinc or zinc alloy coating has been applied 15 to the steel wire at some stage prior to the reduction of the wire to finished size, and after coating it is reduced to the finished size, by drawing down in subsequent passes.

In the wire drawing process, efficient die lubrication is effected with solid or semi-solid lubricants, such as dry sodium soap, greases, mixtures of greases with lime or certain other substances, metallic stearates alone, or metallic stearates mixed with other materials.

25 But in all cases where such lubricants are used in the drawing passes, the drawn wire is coated, wholly or partly, with a strongly adherent film which is usually of dull colour. This discolouration detracts from the appearance of the wire and the presence of the film results in difficulties in certain after treatment to which the wire may have to be subjected.

If certain liquid lubricants instead of plastic or hard lubricants be used, the surface of the 35 wire is not substantially injured by the presence of a film derived from the lubricant. But in this case efficient lubrication is not obtained.

The object of this invention is to provide a 40 process whereby "galvanized" wire, which is efficiently lubricated with the abovementioned plastic lubricants or hard lubricants in the drawing passes may be finished in a final drawing stage or stages and delivered therefrom in bright and clean condition.

45 In carrying out the invention in manufacturing conditions steel rod or steel wire in a size substantially larger than that required in the finished wire is first galvanized. This zinc or zinc alloy coated wire is then drawn down, using an efficient lubricant of plastic or hard nature in all the passes through the dies, except the final pass or passes. Preceding the final pass or passes, steam, hot water, or hot aqueous solution or emulsion is applied to the wire stock and/or the die or dies. The film of lubricant acquired in the earlier passes is cleaned off in the final pass or passes, leaving the wire as it emerges from the final die with a clean and highly polished surface.

In addition to removing the lubricant coating acquired by the wire in the early passes, the steam, hot water, hot aqueous solution or hot emulsion raises the temperature of the wire as the wire passes into the die, and renders the zinc more amenable to the drawing operation, as its ductility is increased with temperature.

The solvent agent is preferably applied by circulating it through chambers intermediate successive dies, that is to say, a chamber intermediate the final die and the penultimate die and if desired also another chamber between the penultimate die and the die preceding it in the series. The wire goes through the solvent flooded chamber or chambers in its course to the final dies.

But other methods of subjecting the wire to the softening or solvent action of the fluids may be used, as the particular method of application of the fluid is a matter of convenience and it is therefore subject to variation.

What I claim as my invention and desire to secure by Letters Patent is:—

1. A multistage process of drawing steel wire which is coated with zinc or zinc alloy, consisting in applying dry or plastic lubricants to the wire only in the drafts preceding the final draft or drafts, and in the final draft stage or stages applying to the wire a fluid which has a solvent or softening action on the surface film of discolored lubricant which has adhered to the wire in the earlier lubricating drafts so as to procure removal of the said film in the final drawing stage or stages.

2. A multistage process of drawing steel wire which is coated with zinc or zinc alloy, consisting in applying dry or plastic lubricants to the wire in the drafts preceding the final draft stage or stages and applying to the wire in the final draft stage or stages a hot fluid which has a solvent or softening action on the surface film of discolored lubricant which has adhered to the wire in the earlier lubricating drafts so as to procure removal of the said film in the final drawing stage or stages.

3. A multistage process of drawing steel wire which is coated with zinc or zinc alloy, consisting in applying dry or plastic lubricants to the wire only in the drafts preceding the final draft or drafts, and in the final draft stage or stages, applying to the wire steam or hot aqueous liquid solution or hot emulsion which liberates the surface film of discolored lubricant which has adhered to the wire in the earlier lubricating drafts, so as to procure removal of the said film in the final drawing stage or stages.

FRANK JENKS.